# EUROPEAN PATENT APPLICATION

(11) **EP 1 607 996 A2**
(43) Date of publication of application: **21.12.2005**
(21) Application number: 05253418.7
(22) Date of filing: 03.06.2005
(51) Int. Cl.: H01J 9/227

(54) **Method of manufacturing phosphor layer structure**

(30) Priority: 17.06.2004 KR 2004045046
(71) Applicant: Samsung SDI Co., Ltd., Suwon-si, Gyeonggi-do (KR)
(72) Inventor: Heo, Jung-na, c/o Samsung Adv. Inst. of Technology, Yongin-si Gyeonggi-do (KR); Jeong, Tae-won, Jungnang-gu Seoul (KR); Park, Shang-hyeun, Boryeong-si Chungcheongnam-do (KR); Kim, Jong-min, 641-1802 Sinnamusil, Suwon-si Gyeonggi-do (KR)
(74) Representative: Kyle, Diana

(57) **Abstract**

Provided is a method of manufacturing a phosphor layer structure including an improved process for forming a phosphor layer between barriers on an anode substrate. The method includes preparing a substrate (11) having inner spaces (12) divided by barriers (13); forming a sacrificial layer (15) on the barriers and the inner spaces to planarize an upper surface of the substrate; forming a phosphor layer (17R, 17G, 17B) on the sacrificial layer (15); and removing the sacrificial layer (15) so that the phosphor layer (17R, 17G, 17B) can be located in the inner spaces (12).

## Description

The present invention relates to a method of manufacturing a phosphor layer structure adopted in devices such as field emission displays (FEDs), and more particularly, to a method of manufacturing a phosphor layer structure having an improved process of forming a phosphor layer between barrier ribs of an anode substrate.

Recently, in the field of display devices, ongoing efforts are focused on developing flat panel displays that have large screens and require increasingly less space for installation.

Types of flat panel displays include a liquid crystal display (LCD), a plasma display panel (PDP), and a field emission display (FED). The FED displays characters and images using a backlight. In the FED, a strong electric field is applied from a gate electrode to emitters that are arranged on a cathode electrode and spaced apart by predetermined intervals to make the emitters emit electrons. The electrons are caused to collide with a phosphor layer coated on the surface of an anode substrate which results in light emission. Here, if the phosphor layer is formed uniformly, brightness, contrast, and color purity are improved.

In the FED, optical interference between different colored phosphors should be minimized. Thus, U.S. Patent No. 6,022,652 (entitled "High Resolution Flat Panel Phosphor Screen with Tall Barriers," published on February 8, 2000) discloses an anode substrate having a barrier structure. In a case where barriers are disposed on the anode substrate and phosphors are formed in spaces between the barriers, the barriers can help maintain color purity and contrast.

In addition, in the above FED, the uniform application of the phosphor largely affects the brightness, contrast, and color purity.

In the above FED adopting an anode substrate having a barrier structure, the presence of the barriers makes it difficult to apply the phosphors between the barriers uniformly. A phosphor layer can be formed by applying a phosphor slurry by spin coating or screen printing. However, it is difficult to uniformly apply the phosphor to spaces between the barriers using these methods.

Alternatively, the phosphor layer can be formed using a dry film-type phosphor. The process of forming the phosphor layer using the dry film-type phosphor will now be described with reference to FIGS. 1A through 1D.

A substrate 1 includes barriers 3 that are formed as protruding stripes separated by predetermined intervals. Between the barriers 3, an inner space is formed, and red (R), green (G), and blue (B) phosphor layers are formed in neighboring inner spaces through processes that will be described later. A phosphor layer 5R of a predetermined color, for example, red, is located on the substrate 1 (FIG. 1A).

Then, the phosphor layer 5R is made to cover the barriers 3 and the inner space on the substrate 1 by use of a blade or a heating roller (FIG. 1B). Next, as shown in FIG. 1C, a mask 7 having a predetermined pattern 7a is located on the phosphor layer 5R and exposure and development processes are performed. As shown in FIG. 1D, through these processes, all portions of the phosphor layer except where the R phosphor layer 5R will be formed are removed. Thus, the red phosphor layer 5R is formed on the substrate 1 in a predetermined pattern.

The processes used to form the red phosphor layer 5R are repeated to form a green phosphor layer and a blue phosphor layer, thus the phosphor layer structure including the red, green, and blue phosphor layers 5R, 5G, and 5B is completed, as shown in FIG. 2. Here, the phosphor layers can be formed uniformly in the inner spaces between the barriers. However, since the dry film-type phosphor used is expensive, as is equipment used to perform the processes, the phosphor layer structure is expensive to manufacture. In addition, it is difficult to form the phosphor layer as a thin film.

The present invention provides a method of manufacturing a phosphor layer structure that involves simplified processes and enables a phosphor layer to be formed on a substrate uniformly.

According to an aspect of the present invention, there is provided a method of manufacturing a phosphor layer structure including: preparing a substrate having inner spaces divided by barriers; forming a sacrificial layer on the barriers and the inner spaces to planarize an upper surface of the substrate; forming a phosphor layer on the sacrificial layer; and removing the sacrificial layer so that the phosphor layer can be located in the inner spaces.

The above and other features and advantages of the present invention will become more apparent by describing in detail exemplary embodiments thereof with reference to the attached drawings in which:
FIGS. 1A through 1D are schematic views of processes of manufacturing a conventional phosphor layer structure;
FIG. 2 is a partial cross-sectional view showing a phosphor layer structure manufactured through the processes shown in FIGS. 1A through 1D;
FIGS. 3A through 3D are schematic views illustrating processes of manufacturing a phosphor layer structure according to an embodiment of the present invention;
FIG. 4 is an electron microscope image showing a phosphor layer structure before being baked, corresponding to the process shown in FIG. 3A;
FIG. 5 is an electron microscope image showing a plan view of the phosphor layer structure after being baked, corresponding to the process shown in FIG. 3D; and
FIG. 6 is an electron microscope image showing a cross-section of the phosphor layer structure after being baked, corresponding to the process shown in FIG. 3D.

Referring to FIGS. 3A through 3D, processes of manufacturing a phosphor layer structure according to an embodiment of the present invention will be described.

As shown in FIG. 3A, a substrate 11 including inner spaces 12 that are divided by barriers 13 is prepared. Here, the substrate 11 can be used as a display device such as a field emission display (FED), in which case the substrate 11 is used as an anode and formed of a material that can transmit incident light.

The substrate 11 and the barriers 13 can be formed of the same material or of different materials. It is desirable that the barriers 13 are formed to a height of 10 ~ 200µm from the surface of the substrate 11 in consideration of color purity and contrast, when the phosphor layer structure is adopted in the display.

As shown in FIG. 3B, a sacrificial layer 15 is formed in the inner spaces 12 and the barriers 13 to planarize an upper surface of the substrate 11.

It is desirable that the sacrificial layer 15 is formed of a thermoplastic resin or a thermosetting resin that is initially fluid. Thus, when first applied, the sacrificial layer 15 flows into and fills the inner spaces 12. Later the sacrificial layer is hardened by heat or light, and finally is removed at a predetermined temperature or by plasma.

The sacrificial layer 15 can be formed of at least one material selected from a group of thermoplastic resins including acrylonitrile- butadiene - styrene terpolymer (ABS), acetal, cellulose-based material, nylon (PA), polybutylene terephthalate (PBT), polycarbonate (PC), polyethylene (PE), polymethyl methacrylate (PMMA), polyphenylene oxide (PPO), polypropylene, polystyrene, polysulfone (PSF), polyvinyl chloride (PVC), polystyrene- acrylonitrile (SAN), and polyvinyl alcohol (PVA).

In addition, the sacrificial layer 15 can be formed of at least one material selected from a group of thermosetting resins including alkyd resin, epoxy resin, melamine resin, phenol- formaldehyde resin, phenolic resin, polyester, silicones, urea- formaldehyde resin, and polyurethane.

As described above, if the sacrificial layer 15 is applied on the substrate 11 in fluid state, it fills the inner spaces 12 and the upper surface of the substrate 11 is planarized. In addition, when the sacrificial layer 15 is hardened by processes of heating or photo irradiation, the planarized upper surface becomes a solid or a gel.

Then, as shown in FIG. 3C, phosphors of red (R), green (G), and blue (B) colors 17R, 17G, and 17B are applied on the sacrificial layer 15. The phosphors 17R, 17G, and 17B can be applied by a spin coating method in which a predetermined amount of phosphor slurry is located on the sacrificial layer 15 and rotated, a printing method in which phosphors are printed onto the sacrificial layer 15, or a slant application method in which the substrate 11 is inclined so that the phosphors can be applied due their own weight. Alternatively, the phosphors 17R, 17G, and 17B can be formed by a dipping method in which the substrate 11 is dipped in a container having the phosphor therein. In FIG. 3C, the phosphors 17R, 17G, and 17B are formed by the spin coating method using particles that are 3 ~ 5µm in diameter, to form a dual-layered structure.

After the phosphors 17R, 17G, and 17B are applied, the layers are dried to complete the phosphor forming process on the sacrificial layer 15.

On the other hand, the phosphor is not applied on the entire upper surface of the substrate. It is desirable that the phosphor is selectively applied on portions of the sacrificial layer 15 corresponding to the upper portion of the inner space on the substrate 11. Also, the phosphors 17R, 17G, and 17B respectively occupy different portions according to their color, and processes for forming the phosphors are performed with respect to color.

After that, the sacrificial layer 15 is removed so that the phoshphors 17R, 17G, and 17B that are located on the sacrificial layer 15 can descend into the corresponding inner spaces 12 as shown in FIG. 3D. Then, the processes of manufacturing the phosphor layer structure of a uniform thin film are completed. Here, the sacrificial layer 15 is removed by baking or conversion to a plasma state in an air atmosphere.

FIG. 4 is an electron microscope image showing the phosphor layer structure before it is baked, corresponding to the process shown in FIG. 3C. That is, FIG. 4 shows the sacrificial layer 15 that is formed in the inner spaces 12 and the barriers 13 after forming the barriers 13 of aluminium on a glass substrate, and the phosphor 17 formed on the sacrificial layer 15. Here, the sacrificial layer 15 is formed of an ethyl cellulose and the phosphors are formed by the dipping method, as an example.

FIGS. 5 and 6 are electron microscope image showing a plane and a cross section of the phosphor layer structure after baking the structure according to the process shown in FIG. 3D. As shown in FIGS. 5 and 6, the phosphor 17 located on the sacrificial layer 15 is formed in the inner spaces 12 between the barriers when the sacrificial layer 15 is removed by baking.

According to the above method of manufacturing the phosphor layer structure of the present invention, the manufacturing processes can be simplified, and the phosphor can be applied uniformly on the substrate having the barriers. Thus, when the phosphor layer structure is manufactured by the above method and a display device such as an FED is fabricated using the phosphor layer structure, the color purity of pixels can be improved.

## Claims

1. A method of manufacturing a phosphor layer structure comprising:
preparing a substrate (11) having inner spaces (12) divided by barriers (13);
forming a sacrificial layer (15) on the barriers (13) and the inner spaces (12) to planarize an upper surface of the substrate (11);
forming a phosphor layer (17R, 17G, 17B) on the sacrificial layer (15); and
removing the sacrificial layer (15) so that the phosphor layer (17R, 17G, 17B) can be located in the inner spaces (12).

2. The method according to claim 1, wherein the sacrificial layer (15) is made of a fluid that is hardened by heat or light and can be removed at a predetermined temperature or by plasma.

3. The method according to claim 2, wherein the sacrificial layer (15) is formed of a thermoplastic resin.

4. The method according to claim 3, wherein the sacrificial layer is formed of at least one material selected from acrylonitrile- butadiene - styrene terpolymer (ABS), acetal, cellulose-based material, nylon (PA), polybutylene terephthalate (PBT), polycarbonate (PC), polyethylene (PE), polymethyl methacrylate (PMMA), polyphenylene oxide (PPO), polypropylene, polystyrene, polysulfone (PSF), polyvinyl chloride (PVC), polystyrene- acrylonitrile (SAN), and polyvinyl alcohol (PVA).

5. The method according to claim 2, wherein the sacrificial layer is formed of a thermosetting resin.

6. The method according to claim 5, wherein the sacrificial layer is formed of at least one material selected from alkyd resin, epoxy resin, melamine resin, phenol- formaldehyde resin, phenolic resin, polyester, silicones, urea- formaldehyde resin, and polyurethane.

7. The method according to any of claims 1 to 6, wherein the barrier is formed to a height of 10 ~ 200µm.

8. The method according to any of claims 1 to 7, wherein the forming of the phosphor layer comprises:
applying phosphor onto the sacrificial layer (15) by a spin coating method, a printing method, a slant application method, or a dipping method; and
drying the applied phosphor.

9. The method according to claim 8, wherein the phosphor is applied on a part of the sacrificial layer (15) that corresponds to an upper portion of the inner spaces (12) of the substrate (11).
